

Oct. 20, 1931.

W. H. MILLSPAUGH

1,828,335

CENTRIFUGAL CASTING METHOD

Filed April 26, 1929 2 Sheets-Sheet 1

Fig. 1.



Fig. 2.



Fig. 3.



Fig. 4.



INVENTOR

William H. Millspaugh

BY

Marshall & Hawley

ATTORNEYS

Oct. 20, 1931.

W. H. MILLSPAUGH  
CENTRIFUGAL CASTING METHOD

1,828,335

Filed April 26, 1929

2 Sheets-Sheet 2

Fig. 5.



Fig. 6.



Fig. 7.



INVENTOR  
William H. Millspaugh  
BY  
Marshall & Hawley  
ATTORNEYS

## UNITED STATES PATENT OFFICE

WILLIAM H. MILLSPAUGH, OF SANDUSKY, OHIO, ASSIGNOR TO THE PAPER & TEXTILE MACHINERY COMPANY, OF SANDUSKY, OHIO, A CORPORATION OF OHIO

## CENTRIFUGAL CASTING METHOD

Application filed April 26, 1929. Serial No. 358,231.

This invention relates to improvements in centrifugal casting and more particularly to a method of controlling the rate of dissipating the heat of the molten metal poured into a rotatable mold. The invention relates specifically to the method of cooling the molten metal at different desired rates by providing molds of different heat dissipating properties as by the use of molds of different wall thickness for castings of different thickness or of different metals or materials.

It is well known that the problems connected with the cooling of centrifugal castings such as tubular or substantially cylindrical articles, are much more complex than the problems of cooling floor castings. The heat of the metal poured into rotatable molds is dissipated both inwardly and outwardly and with certain metals it is essential to control the rate of the outward heat dissipation for if it is too rapid the metal will crack and if it is too slow, the desired character of metal in the casting will not be produced. I have discovered that by the simple expedient of proportioning the thickness of the wall of the mold to the thickness of the casting made therein, the rate of cooling can be controlled, and that by using thicker mold walls for thicker castings and vice versa, the former difficulties are overcome.

The molds used in the rotors of centrifugal casting machines are removable and interchangeable so that as soon as a casting has set, it, with its mold, may be removed from the rotor and another mold of the same or different type inserted. The casting is cooled within its mold but not necessarily within the rotor of a casting machine. According to this invention castings of many different diameters and wall thicknesses may be made in one rotor. I am aware of the fact that it has been suggested in general terms, that castings of different sizes may be produced in one machine, but this has not been accomplished practically because it has not been known that merely changing the internal diameter of the mold to get castings of different external diameters, is not enough to get good results. But I have found that for a casting of a given thickness, a certain mold wall

thickness is required, regardless of the outside diameter of the casting, also that for castings of different thickness but of the same outside diameter, different mold wall thicknesses are needed.

In order to more clearly disclose my invention, drawings are submitted to illustrate diagrammatically various ways of practicing the novel method. All of the drawings are transverse sections taken through a rotor, a mold and a casting, and in each of them the outer member 10 is the same rotor of a centrifugal casting machine. Figs. 1-4 show metallic or "permanent" molds 20A, 20B, 20C and 20D of different diameters and thicknesses, and Figs. 5-7 show compound molds comprising refractory lined core-cases, these compound molds being of different diameters and thicknesses.

Figs. 1, 2 and 3 show three castings A, B and C of the same outside diameter but of different thicknesses. The mold 20A for the thinnest casting A has a thinner wall than the mold 20B for the thicker casting B, and the mold 20C for the thickest casting C, has the thickest wall. Each of these molds is provided with spacing ribs 21A, 21B and 21C or equivalent elements which serve the two-fold function of making each of the molds fit the same rotor, and of providing an insulating air space between the outside of the mold and the inside of the rotor.

Fig. 4 illustrates a large diameter thin casting D on a thin walled mold 20D, spaced from rotor 10 by ribs 21D. It is obvious that a great variety of other sizes of castings of different thicknesses may be made in the same rotor according to this principle.

The method may be practiced also with refractory molds as shown in Figs. 5-7. In these figures each comprise a metallic shell which I call a "core-case" and a liner of sand or other refractory material.

In Figs. 5 and 6 the same core-case is shown. It comprises a body 30 with spacing ribs 31, or equivalent elements, which are similar to and serve the same purpose as the ribs in the previous figures, and perforations 32 for the escape of gases from the refractory material into the spaces between the outside of the

core-case and the inside of the rotor. A thin walled casting of large diameter is shown at E in Fig. 5. This is cast on a refractory liner 33, the thickness of which together with the thickness of the core-case is comparatively thin. That is the thickness of this compound mold is proportioned to give the desired rate of heat radiation and dissipation for such a casting as that shown at E.

- 10 The casting F shown in Fig. 6 is of smaller diameter and has a thicker wall than that shown in Fig. 5. In this case a thicker refractory liner 33A is used. It has been assumed heretofore that a casting of the diameter of casting F and no thicker than casting E could be made in the mold shown in Fig. 6, and this assumption has been the reason for the non-development of making castings of different diameters in the same machine, 15 for with some metals and under usual conditions this cannot be done. However, Figs. 5 and 6 show that castings of different diameters may be made in the same core-case.

When it is desired to make a casting of the same diameter as casting F and of the thickness of casting E, a different core-case must be used as shown at 30A in Fig. 7. G designates such a casting and 33B its refractory liner. The combined thickness of the core-case 30A and its liner 33B in Fig. 7 is slightly less than the thickness of the compound mold 20, 33 of Fig. 5 because there is less metal in casting G than there is in casting E. This showing is based upon the assumption that 25 castings G and E are of the same metal and are poured at the same temperature. Of course variations in the mold wall thicknesses are made to meet the requirements of the metals and pouring temperatures used.

- 30 What I claim is:

1. The herein described method of making hollow centrifugal castings which comprises providing for outward heat dissipation from molten metal poured into rotatable molds and 45 controlling the rate of said outward heat dissipation, by proportioning the dimensions of the mold walls in accordance with the character of the castings made therein, to establish the heat conducting characteristics of the 50 molds.

2. The herein described method of making hollow centrifugal castings of uniform wall thicknesses which comprises providing for a uniform outward heat dissipation from molten metal poured into rotatable molds and controlling the rate of said outward heat dissipation, by proportioning the thickness of the mold walls in accordance with the character of the castings made therein, to establish the heat conducting characteristics of the 55 molds.

3. The herein described method of making hollow centrifugal castings of uniform wall thicknesses which comprises providing for a 60 uniform outward heat dissipation from mol-

ten metal poured into rotatable molds and controlling the rate of said outward heat dissipation, by proportioning the thickness of the mold walls in accordance with the thickness and material of the castings made therein, to establish the heat conducting characteristics of the molds. 70

4. The herein described method of making hollow centrifugal castings of uniform wall thicknesses which comprises providing for a 75 uniform outward heat dissipation from molten metal poured into rotatable molds and controlling the rate of said outward heat dissipation, by providing molds having walls of homogeneous heat conductivity and proportioning the thickness of said walls in accordance with the thickness and material of the castings made therein, to establish the 80 heat conducting characteristics of the molds.

In witness whereof, I have hereunto set 85 my hand this 3rd day of April, 1929.

WILLIAM H. MILLSPAUGH.

90

95

100

105

110

115

120

125

130